

April 21, 1931.

C. GOTTWALD

1,801,500

WATER REPELLENT PACKING MATERIAL

Filed Aug. 12, 1927



Inventor

Christian Gottwald

Ross Hudson & Kent  
attns

## UNITED STATES PATENT OFFICE

CHRISTIAN GOTTLWALD, OF CLEVELAND, OHIO, ASSIGNOR TO THE RIC-WIL COMPANY, OF CLEVELAND, OHIO, A CORPORATION OF OHIO

WATER-REPELLENT PACKING MATERIAL

REISSUED

Application filed August 12, 1927. Serial No. 212,502.

The present invention relates to an improvement in underground conduit systems, in which a pipe or pipes for conveying a liquid or gas are housed within an enveloping structure of metal, tile, concrete or brick.

The invention has particularly to do with the matter of packing for surrounding the pipe or pipes within the housing or envelope, the packing having the peculiar property of 10 repelling water, so that the same will not become water-soaked, and thus break down its qualities as a thermo non-conductor.

Reference should be had to the accompanying drawing forming a part of this specification, in which the figure shows, in cross section, a well known form of underground conduit construction with the thermo non-conducting packing surrounding the enclosed pipe.

20 In the drawing, 1 and 2 designate the upper and lower portions of a well known form of conduit, usually made of vitreous material. A well known form of base drain is indicated at 2.

25 Within the conduit is a pipe 4 for fluid conducting purposes, which pipe is supported upon supports 5 which are of a well known commercial form.

Surrounding the pipe and confined within 30 the conduit is the thermo non-conducting packing material to which reference is made later on in this specification.

Underground conduit systems are prone to have moisture accumulate within the outer 35 casing or conduit, either because of moisture condensing, or in some instances from the ingress of water from the outside.

It is usual in underground conduit systems to provide some sort of draining feature, both to drain water from the surrounding earth in which the conduit is placed, and also to provide suitable vents or means by which water that may accumulate or find its way into the conduit itself may be drained.

45 In underground conduit systems where the pipe or pipes are conveying a liquid or gas which is either above or below the normal temperature, as for instance steam, or on the other hand a refrigerant gas or fluid, it is 50 necessary to enclose and pack the pipe or pipes

with some suitable non-conductor of heat. The difficulty has been that the usual forms of thermo non-conductors become impregnated with water or moisture, and thus decrease, and with the accumulation of sufficient moisture break down the thermo non-conductivity of the packing. The usual packings which have heretofore been employed, such as shredded asbestos, rock wool and mineral wool are in each instance comprised of siliceous fibers which of themselves are water-proof. These substances being crystalline in structure and not cellular will not absorb water, so that they may be properly described as water-proof. However, when these substances are used as packing materials in underground conduit systems, the water which condenses within the conduit or finds its way into the conduit from outside sources will nevertheless soak the fibrous mass, the water finding its way into the interstices between the fibers and there being held, and upon a sufficient accumulation of water the thermo non-conductivity of the packing mass is impaired or destroyed. Apparently the water 70 penetrates into the mass of fibers by capillarity and lodges in the interstices between the fibers, and this will occur even though care is taken to sufficiently pack the fibrous mass so as to avoid leakage or appreciable 75 pockets in the packing.

The present invention has to do with a packing material, which, by treatment, is rendered water repellent, and by this is meant that water coming in contact with a 80 mass of fibers is repelled, so that the water does not find its way into the interstices between the fibers.

More specifically speaking a fibrous packing material, such as shredded asbestos, rock 90 wool, mineral wool or equivalent material which in usual commercial form is unmatted and having loosely associated fibers which, in itself, is water-proof, is treated by chemicals so as to render the fibers water repellent, and when a mass of unmatted, loosely associated fibers of material so treated is loosely packed around a pipe or pipes within a conduit, the density of the packing being such as to avoid 95 appreciable sized pockets or spaces in the 100

- packing, water coming in contact with the mass of fibrous material will be repelled and the water will run down the inner wall of the enveloping conduit to be discharged through the usual base drain. The effect of the treatment given to the fibers of the fibrous material seems to be in effect to break down the usual capillary action, by which water might ordinarily be drawn into the interstices between the fibers, and by virtue thereof the water is repelled. Whether the foregoing be the correct explanation of the phenomena is not important, but the fact that the fibers are rendered repellent to water is important.
- 15 The fibrous material may be treated, to render it water repellent, by various substances, one of which may be mentioned being a five to ten percent solution of aluminum stearate, this specific substance being not included in the present invention but forming the subject matter of a copending application, filed in the name of Carl A. Black, Serial No. 212,604, filed August 12, 1927.

I am aware that it has been heretofore proposed to treat certain material which is cellular in nature in order to make it water-proof, but my invention differs from such procedure in that it makes the fibrous material treated water repellent.

25 Merely being water-proof is not sufficient, for, as before pointed out, asbestos, rock wool and mineral wool are all inherently water-proof, but nevertheless a fibrous mass of these materials will water-soak by the accumulation of water in the interstices between the fibers.

30 It is only by making the fibers water repellent so that water will not accumulate in the interstices between the fibers, that an efficient packing for underground pipes which are housed in conduits can be obtained.

35 Having thus described my invention what I claim as new is:

1. The combination with a conduit having drainage means and a fluid conducting pipe therein, of a mass of thermo-non-conducting material comprising a mass of unmatted and comparatively loosely associated mineral fibers coated with material which renders them water repellent, surrounding said pipe and within the conduit.

40 2. The combination with a conduit having drainage means and a fluid conducting pipe therein, of a mass of thermo-non-conducting material comprising a mass of unmatted comparatively loosely associated asbestos fibers coated to render them water repellent surrounding said pipe and within the conduit.

45 In testimony whereof, I hereunto affix my signature.

50 CHRISTIAN GOTTWALD.